# EUROPEAN PATENT SPECIFICATION

(11) **EP 0 209 538 B1**
(45) Date of publication and mention of the grant of the patent: **23.05.1990**
(21) Application number: 86900327.7
(22) Date of filing: 10.12.1985
(51) Int. Cl.: D21H 17/68

(54) **PROCESS FOR MANUFACTURE OF PAPER HOLDING CLAY OR OTHER FILLERS**
VERFAHREN ZUR HERSTELLUNG VON TONERDE UND ANDEREN FÜLLMATERIALIEN ZUM VERSTÄRKEN VON PAPIER
PROCEDE DE PRODUCTION D'ARGILE ET D'AUTRES CHARGES DE CONSOLIDATION DE PAPIER

(30) Priority: 15.01.1985 SE 8500162
(43) Date of publication of application: 28.01.1987
(73) Proprietor: MO OCH DOMSJÖ AKTIEBOLAG, S-891 91 Örnsköldsvik (SE)
(72) Inventor: GAVELIN, Gunnar, S-183 51 Täby (SE)
(74) Representative: Barz, Peter, Dr.
(86) International application number: SE8500514
(87) International publication number: WO8604370

(56) References cited:
- FR-A- 2 173 928
- US-A- 3 141 815
- US-A- 3 865 686
- US-A- 4 295 933
- Pulp Technol & Treatment for Paper (1978), Miller Freeman Publns p 16o, 177-179, 257-26o, 277-28o, 664, 676-677.
- Journal of Pol Sci: Pol Lett Ed, Vol 2o, 615-62o (1982), Alince, B, et al "Cationic Latex in Fiber-Clay Paper Composites".
- Tappi J (1983): 1, 92-95, Alince, B, et al "Intraction of cationic clay particles with pulp fibers".
- Tappi J: 66 (1983): 3, 137-139, Waech, T G, "Improving filler retention by adding filler after retention and addition".
- Tappi J 65 (1982): 4, 95-99, Tanaka H, et al "How retention-aids change the distribution of filler in paper".
- Svensk papperstidning 1983: 1o, p. 4o-41, 44, 47-48, 51, Fineman I.

## Description

This invention can be used to improve the retention of fillers during papermaking, to prevent a harmful agglomeration of filler particles in paper and to obtain a uniform distribution of filler in paper. The invention also mitigates the harmful effect of filler on the strength of paper as well as the harmful effect of retention aids on paper formation. Aggregates of filler particles and fines from beaten or refined pulps contribute to a high opacity in the paper.

When paper with a high content of filler is produced, a retention aid is usually added to the pulp suspension in order to improve the retention, which would otherwise become so low that the content of filler in the circulating white water would become too high for safe operation of the machine and would also result in high losses to the sewer.

Such flocculation of filler in a pulp suspension, however, entails an expensive consumption of chemicals and has unwanted secondary effects. Thus the chemical also flocculates the fibers in the pulp and thereby damages the formation of the paper. A fluctuating efficiency of the process can upset the manufacturing processes on the paper machine. In the paper the filler content will be considerably higher on the top side than on the side facing the wire. Agglomeration of filler particles causes a reduction of the light scattering of the paper.

The purpose of this invention is to achieve an improved filler retention without generation of dense filler agglomerates. A solution to this problem has been found to be the process as claimed in Claim 1. Specific embodiments of this process are the subject of Claims 2 to 5. An important feature of the process is to flocculate the filler particles when mixed with a fines fraction of wood fibrils, whereby the particles are kept apart by these fibrils, which latter are bound into voluminous flocs, presumably by polymer bridging, the flocs being easily filtered off during drainage on the paper machine wire and retaining their position in the fibre network in spite of the flow of water through it during dewatering and pressing on the paper machine. Just as the filler particles, the fines have an ability to scatter light and thereby improve the opacity of the paper provided only that a distance of at least one half wave length of the light can be maintained between the fibrils in the paper, something that will be promoted by coflocculation of fines and fillers.

It is essential in this process that the fibrils have a certain stiffness, so that the surface tension will not give too much optical contact between them during drying of the paper. The fibrils should, therefore, preferably derive from mechanical or chemimechanical pulp, in which the fibre wall, from which the fibrils have been peeled off, still retains the stiffness of wood. However, the pulp should preferably be peroxide bleached, since this invention will be used mainly in combination with manufacture of printing paper requiring a high brightness. The coflocculation process itself is just as efficient with fines of chemical pulp, and on a paper machine it is recommended to use the rich white water from the first part of the drainage table for dilution of the fines to be used in the process. This will greatly improve retention and lower the white water consistency. Mechanical pulp for use in high grade printing paper can be made with a fines content above 50%, but one cannot go too far in this respect since long fibres are also needed for strength and since retention will be a problem, when such pulp is added to the furnish. When the above type of pulp is used according to this invention, it will cause no drainage or retention troubles and can be as finely refined as is possible.

If such mechanical pulp is not available or not suitable as an ingredient in the paper being produced, part of the main furnish can be subjected to a separate refining process producing a suitable fine grade pulp. The quantity required amounts to 20% on the weight of the filler added. The refining should take place at a consistency of 20-50% in order to produce fibrils and lamellas rather than broken fibres.

For this refining many conventional refiners can be used but means should preferably be provided for recirculation of pulp. Filler may be added to the pulp during this process in order to get a good mixing, but this is not essential.

The fine grade pulp, which conveniently can be a commercial mechanical pulp of very lowfreeness, for example 50 ml C.S.F. (Canadian Standard Freeness), is diluted in an agitated tank preferably with white water from the first part of the drainage table to a consistency of conveniently 57-10 g/I. The pulp is then mixed with a filler suspension at a rate giving for example 20% fines on the weight of the filler, which is conveniently achieved by continuous pumping of the two suspensions into a mixing chamber. When mixing has been achieved, a retention aid is introduced for coflocculation of fines and filler. The floc suspension is then pumped into the furnish for example ahead of the fan pump feeding the paper machine.

### Description of figures

Figure 1 shows filler distribution through the thickness of two sheets made from coflocculated blends of equal parts of fines and mineral filler.
Figure 2 shows filler retention in a sheet mould as a function of retention aid addition.
   P+F: Filler preflocculated with a fines fraction
   P+P: Filler added to the pulp and then retention aid mixed in.

Figure 1 shows the filler distribution from top side to wire side in two sheets made from equal parts of filler and fines flocculated by a polymer. The picture demonstrates that the filler particles in these sheets were so firmly bound to the fines that they retained their positions in the sheet during drainage, pressing and drying.

Figure 2 shows the results of retention studies on a laboratory sheet mould, in which sheets have been made either after addition of filler and retention aid to the furnish (P+P) or after addition of preflocculated fines-filler aggregates to the sheet machine. (P+F) It is seen that a polymer consumption of 150 g/t during conventional sheet-making gave the same retention as a polymer consumption of 60 g/t during coflocculation of fines and filler.

The following Table presents sediment concentrations of some blends of fines and filler. By far the lowest sediment concentration was obtained by use of the coflocculation process, that is, the most voluminous flocs were formed. The same effect is not obtained if either clay or fines is flocculated before mixing with the other.

The coflocculation process has been tried on a pilot paper machine and the results compared with those obtained after conventional papermaking using the same furnish. The following results were recorded:

Although the coflocculated paper held 8% of a very low freeness groundwood pulp the TEA was 40% higher, an effect which can be explained by a very much better formation and by less interference of the filler particles with fiber-fiber bonding. It is remarkable that this strength increase could be combined with a reduction of the density and an increase of the light scattering. Normally, the latter two properties will deteriorate, when strength goes up. It should be observed that the positive effects of coeffloculation are obtained without any extra expenses for chemicals or pulp.

## Claims

1. A process for manufacturing paper containing clay or other mineral fillers, characterized by mixing a fibre suspension consisting of a fines fraction of wood fibrils with said filler, then coflocculating the fines fraction and filler by adding to the mixture a polymeric retention aid and thereafter continuously feeding the resulting fines-filler flocs into a furnish forwarded to a paper machine.

2. A process according to claim 1, wherein said fines fraction predominantly consists of fibrils from broken down fibre walls of mechanical pulp.

3. A process according to claim 1, wherein said fines fraction is derived from a chemi-mechanical pulp.

4. A process according to claim 1, wherein said fines fraction is derived from a chemical pulp.

5. A process according to any one of claims 1 to 4, wherein said retention aid is a cation active polyacrylamide.

6. A process according to any one of claims 1 to 5, wherein said fibre suspension is diluted with white water from a paper machine.

7. A process according to claim 6, wherein said white water is taken from the early part of the drainage table of a paper machine.

## Patentansprüche

1. Verfahren zur Herstellung von Papier, das Ton oder andere Mineralfüllstoffe enthält, dadurch gekennzeichnet, daß man eine Fasersuspension, die aus einer Siebfeinfraktion von Holzfibrillen besteht, mit dem Füllstoff mischt, dann die Siebfeinfraktion und den Füllstoff durch Zugabe eines polymeren Retentionshilfsmittels zu der Mischung miteinander ausflockt und danach einen Stoffeintrag, der zu einer Papiermaschine befördert wird, kontinuierlich mit den resultiernden Siebfein-Füllstoffflocken beschickt.

2. Verfahren nach Anspruch 1, worin die Siebfeinfraktion hauptsächlich aus Fibrillen aus zerkleinerten Faserwänden von mechanischem Halbstoff besteht.

3. Verfahren nach Anspruch 1, worin die Siebfeinfraktion von einem chemi-mechanischen Halbstoff abstammt.

4. Verfahren nach Anspruch 1, worin die Siebfeinfraktion von einem chemischen Halbstoff abstammt.

5. Verfahren nach irgend einem der Ansprüche 1 bis 4, worin das Retentionshilfsmittel ein kationsaktives Polyacrylamid ist.

6. Verfahren nach irgend einem der Ansprüche 1 bis 5, worin die Fasersuspension mit Siebwasser von einer Papiermaschine verdünnt wird.

7. Verfahren nach Anspruch 6, worin das Siebwasser von dem ersteren Teil des Entwässerungstisches einer Papiermaschine genommen wird.

## Revendications

1. Procédé de fabrication de papier contenant de l'argile ou autres charges minérales, caractérisé par le fait qu'on mélange une suspension de fibres consistant en une fraction de particules fines de fibrilles de bois avec cette charge, puis on effectue la co-floculation de cette fraction de particules fines et de fibres en ajoutant au mélange un polymère comme adjuvant de rétention et ensuite on envoie en continu les flocons résultants de particules fines et de charge dans un système d'alimentation de machine de fabrication de papier.

2. Procédé selon la revendication 1, caractérisé par le fait qu'une fraction de particules fines consiste principalement en fibrilles de parois de fibres brisées d'une pâte mécanique.

3. Procédé selon la revendication 1, caractérisé par le fait que la fraction de particules fines provient d'une pâte chimico-mécanique.

4. Procédé selon la revendication 1, caractérisé par le fait que la fraction de particules fines provient d'une pâte chimique.

5. Procédé selon l'une quelconque des revendications 1 à 4, caractérisé par le fait que l'adjuvant de rétention est un polyacrylamide cationiquement actif.

6. Procédé selon l'une quelconque des revendications 1 à 5, caractérisé par le fait que l'on dilue la suspension de fibres par de l'eau blanche d'une machine de fabrication de papier.

7. Procédé selon la revendication 6, caractérisé par le fait que l'on prélève l'eau blanche de la partie antérieure de la table de drainage d'une machine de fabrication de papier.
